

## UNITED STATES PATENT OFFICE

LINN BRADLEY, OF MONTCLAIR, NEW JERSEY, AND EDWARD P. MCKEEFE, OF PLATTSBURG, NEW YORK, ASSIGNEES TO BRADLEY-MCKEEFE CORPORATION, OF NEW YORK, N. Y., A CORPORATION OF NEW JERSEY

## MANUFACTURE OF PULP, ETC.

No Drawing.

Application filed April 4, 1924. Serial No. 704,176.

This invention relates to improvements in the production of chemical pulp from woods (both coniferous and non-coniferous) whereby good yields of chemical pulp can be obtained, and whereby woods, which are ordinarily considered of little or no value for the production of chemical pulp which can be readily bleached to a high white by the usual commercial bleaching methods, and for the production of papers of high quality, can be advantageously utilized for the production of chemical pulp therefrom.

This invention includes a new cooking liquor for the cooking of woods, as well as the new and improved pulp-making or cooking operation itself for the production of the pulp from the wood; and it includes the residual liquors produced by the pulp-making operation; and it includes the new pulps and the new papers made therefrom. It also includes a new and improved method of regeneration of the cooking liquor, and improvements in the process of treating the residual liquors; as well as a complete regenerative process for the regeneration of the cooking liquor and the carrying out of successive cooking operations with regenerated cooking liquor; the details of which are hereinafter more fully set forth.

In our prior application, Serial No. 481,147, filed June 28, 1921, we have described an improved process of producing chemical pulp from woods in which the woods are subjected to a cooking operation with a cooking liquor containing essentially a normal alkali sulphite, either alone or with a small amount of caustic soda, etc.

In the process of making chemical pulp from wood, according to the present invention, the wood may be freed from bark, chipped and then subjected to a cooking operation under pressure and at an elevated temperature with a cooking liquor containing essentially a normal alkali sulphite and an alkali thiosulphate, the sulphite generally being in preponderating amount. The cooking liquor may contain moderate amounts of other constituents such as sodium carbonate, etc., but we have found the process an ad-

vantageous one when such other constituents are substantially absent.

We have found that chemical pulp can be produced from woods of various kinds by cooking the wood chips with a cooking liquor containing both normal sodium sulphite and sodium thiosulphate, and that a satisfactory pulp can be thus produced which can be commercially bleached, provided sodium sulphite is present in sufficient amount. This result is surprising in view of the fact that, for example, when aspen chips are cooked with a cooking liquor composed essentially of a solution of sodium thiosulphate the resulting pulp is of a very dark color and very difficult to bleach, and the pulp is of an entirely different character. We do not claim in this application the cooking of wood with a cooking liquor composed essentially of a solution of sodium thiosulphate, as this is being included in a separate application.

The cooking liquor containing both the normal sodium sulphite and sodium thiosulphate may advantageously be produced from the residual liquor from the cooking operation, in one or another of the various methods of treatment hereinafter described. The cooking liquor can, however, be produced in the first instance in any suitable manner, and additional amounts required to supplement or modify that regenerated from the residual liquors may also be supplied in any suitable manner. For example, solutions containing sodium carbonate and a small amount of sodium sulfide or polysulfide can be treated with sulfur dioxide or sodium bisulfite or both with resulting reaction of the sulfur dioxide with the sodium carbonate to produce sodium sulfite, and with reaction of sulfur dioxide with the sodium sulfide or polysulfide to produce some sodium thiosulfate. Where elementary sulfur (especially when finely divided) is present in or added to the solution treated, this may also react with sodium sulfite to produce some sodium thiosulfate.

In our investigation of the action of sodium thiosulfate in a cooking liquor we have investigated the use of sodium thiosulfate alone as well as its use in conjunction with

sodium sulfite and other materials in varying proportions. We have found for example that non-coniferous woods in general can be readily pulped with a solution of sodium thiosulfate alone if used in sufficient strength. We do not, however, claim this process herein as it forms the subject of a separate application. The pulp produced when sodium thiosulfate is used alone is very dark 5 in color and difficult to bleach, being dark brown or even black after washing, and not being readily bleachable by commercial bleaching methods. The odor from the freshly opened digester is also quite offensive 10 when sodium thiosulfate alone or with caustic soda is used as the cooking liquor. We have also found that if sodium sulfite and sodium thiosulfate are used together for cooking woods, it is difficult or impossible to 15 obtain a commercially bleachable pulp if the amount of sodium thiosulfate is too high and the amount of sodium sulfite is too small. 20

We have found, however, as a result of our investigations, that if the cooking liquor 25 contains a sufficient amount of sodium sulfite, based on the weight of the wood, and the concentration of the liquor and the time and temperature of cooking are suitable, a satisfactory pulp can be obtained even though 30 the cooking liquor contains quite a large amount of sodium thiosulfate. In practice, we have found that an amount of sodium sulfite equivalent to about 30% or more on the bone dry weight of the woods is desirable, 35 and we have used much more than this with excellent results; for example, we have used as much as 50% and even more of sodium sulfite. In general, the amount of sodium thiosulfate should be less than that of the sodium sulfite. For best results we consider 40 that only a relatively small amount of sodium thiosulfate is desirable. For example, where the amount of sodium sulfite is equivalent to at least 30% of the bone dry weight 45 of the wood, the amount of sodium thiosulfate may vary from a few percents up to say 15% of the bone dry wood, or even more sodium thiosulfate may be present, although, as above stated we consider it more advantageous to use a smaller amount, amounting, 50 for example, to only a few percent on the bone dry weight of the wood.

One of the important advantages which the present invention presents is that it is 55 applicable to the treatment of various kinds of woods, both coniferous and non-coniferous, including various woods that are not commonly considered available for the production of satisfactory chemical pulp therefrom. The rapidly decreasing supply of 60 wood suitable and available for pulp-making purposes, according to the usual present day processes, and the high cost of equipment and operation of chemical pulp mills, makes 65 it of industrial and economic importance to

increase the yield of pulp from woods which are commonly used for pulp-making purposes and to make available for pulp-making purposes woods ordinarily considered of little or no value for the production of high 70 grade pulp. The process of the present invention is applicable not only to the common pulp woods, such as poplar and spruce, etc., but also to other woods, both coniferous and non-coniferous, which are not commonly included among the pulp woods. Non-coniferous woods, including the heavy dense hard woods, such as birches, beeches and maples, the different kinds of oak, hickory, eucalyptus, elm, ash, etc., may be used as well as 80 poplars, aspens, bass wood, cotton wood, chestnut, gums, etc. So also coniferous woods including not only spruces, firs, and balsam, but also hemlocks, cedars, cypress, larches, tamarack and the various pines. 85 Pines of a resinous character, such as yellow pines, white pine, jack pine, longleaf pine, shortleaf pine, lodgepole pine, and other similar pines can thus be treated according to the present invention for the production of 90 suitable chemical pulp therefrom.

The cooking operation can be carried out in digesters of the type now used, for example, in the soda or sulfate processes. Where the cooking liquor contains only sodium sulfite and sodium thiosulfate, or only these chemicals together with others which are neutral or alkaline to phenolphthalein, the provision of an acid resistant lining in the digester is not necessary, but ordinary iron or 95 steel digesters (preferably welded) can be used. The digesters may be heated and the cooking liquor circulated therein in any suitable manner. Outside circulation of the cooking liquor from the bottom of the digester with reintroduction at the top through a suitable distributor can be employed and with suitable heating of the cooking liquor which is being circulated. Rotary digesters also may be used with distinct advantage. 100

In carrying out the cooking operation, different temperatures may be employed, for example, a temperature corresponding to saturated steam at pressures up to 180 lbs. to the square inch, gauge reading. The invention presents the advantage that high temperatures, corresponding to gauge pressures around 120 lbs. or higher of saturated steam, can be used without unduly injuring the pulp produced. Temperatures corresponding to around 140 lbs. steam gauge pressure, or even higher, can thus be used in commercial operations. In general, we have found it advantageous to use higher temperatures with coniferous woods than with non-coniferous woods. With non-coniferous woods it is advantageous to use temperatures around 165° C. or higher, and with coniferous woods, temperatures around 175° C. and higher, e. g., around 180 to 190° C. 115

The amounts of sodium sulfite and sodium thiosulfate can be varied. In general, the amount of sodium sulfite should be around 30% or more based on the bone dry weight of the wood treated, and more than this can be used with excellent results; while we consider it desirable that the sodium thiosulfate should be present in considerably less amount than that of the sodium sulfite. It is one advantage of the process of the present invention that the amounts of the chemicals employed can be considerably in excess of that actually required in the process since the excess does not have such an injurious action on the fibres that a similar excess of reactive chemicals has in, for example, the soda process. The amount of sulfite may be e. g. around 40 to 50% of the bone dry weight of the wood, or even higher, e. g., 60% or more, but such large amounts are not necessary.

In carrying out the process of the present invention, the procedure may differ somewhat with non-coniferous woods, and particularly dense hard woods such as birches, beeches, and maples and with less dense woods such as poplars or with coniferous woods such as spruces and pines. With non-coniferous woods, for example, the digester charge can be heated in a relatively rapid manner to the cooking temperature as disclosed in a companion application; while with coniferous woods we find it important to heat up the digester charge gradually so as to secure thorough penetration of the wood chips with the cooking liquor at a temperature below the active cooking temperature, before heating the charge to the active cooking temperature.

When the cooking operation is completed, the charge can be blown in to a blow pit and the pulp washed and subjected to further treatment in the manner customary in the subsequent treatment of chemical pulp either for the manufacture of merchantable pulp or for the manufacture of paper or other products therefrom.

It is an important advantage of the present invention that the yield of pulp obtained is considerably higher than is commonly obtained by the ordinary chemical pulp-making processes. The yield of pulp may be, for example, several per cent more from poplar wood (aspen) than commonly obtained by the ordinary soda process from that wood. We have also found that somewhat increased yields can be obtained from coniferous woods such as spruces and pines, when treated according to the present invention, as compared, for example, with the ordinary acid-sulfite process so-called.

It is a further advantage of the process that heavy woods, such as birches, beeches and maples, oaks, etc., or locust, certain pines, tamarack, etc., can be used even though the weight of a digester charge of these woods is

considerably greater than the weight of a similar charge of poplar or spruce, and even though a correspondingly increased amount of chemical in the cooking liquor is required. With a digester charged with wood chips, the volume of cooking liquor which can be introduced into the digester is limited; and with the soda process, for example, the strength of the caustic soda solution which can be satisfactorily used in the process is also limited. Such dense or heavy woods cannot therefore be quite so satisfactorily cooked by the soda process when the digester is fully charged. In the process of the present invention, however, a digester full of chips obtained from such heavy woods can be satisfactorily cooked, inasmuch as the chemicals used in the process can be used in a sufficiently concentrated solution to bring about the cooking of the entire digester charge, even though the process is carried out at a much higher temperature and pressure than is commonly practiced in the present day pulp-making operations. When such dense heavy woods are used, it should be evident that a greatly increased yield of chemical pulp will be obtained per digester charge of wood.

The pulps produced by the process of the present invention are different in character from the pulps commonly produced by the usual methods, and we accordingly regard the pulps new and improved pulps. They contain characteristic fibres of distinctive feel and possessing great strength. Various pine woods, such as, for example, jack pine, as well as spruce, hemlock and other coniferous woods, when treated according to the process of the present invention, yield pulps of excellent strength. It will be evident, however, that inasmuch as different woods differ in their fibre structures from each other, the pulps produced therefrom will differ somewhat from each other. The process of the present invention accordingly will give different kinds of pulp from different kinds of wood, each wood being more or less characteristic in the pulp which it gives.

Owing to the valuable properties which the pulps produced by the present invention possess, they can be advantageously used for purposes for which other pulps from the same kinds of wood could not be used so satisfactorily.

The present invention as hereinbefore stated is also applicable for the production of a high quality of chemical pulp from various species of woods which heretofore have not been generally considered as pulp woods, or have been considered of little if any value for the manufacture of high grade chemical pulp. In particular, we have found that resinous woods, such as pines of various kinds, can be advantageously treated by our improved process without serious difficulty arising from the resinous constituents which

these woods contain, particularly if the cooking operation is carried out with gradual heating of the digester charge together with adequate liquor circulation over a considerable period of time before it is finally brought to the active cooking temperature and pressure. In the case of various heavy woods, the process of the present invention gives high grade pulps with high yields.

- 10 The residual liquors produced by the process of the present invention are of characteristic composition and properties. Our investigation of the chemical reaction which takes place during the cooking of woods leads us to believe that the wood substance is a complex reactive chemical substance which reacts with the chemicals contained in the cooking liquor, and that the nature of the reaction and of the reaction products produced varies 15 with the cooking liquor employed. When both sodium sulfite and sodium thiosulfate are present in the cooking liquor, both of these chemical substances appear to have a characteristic and distinctive action upon the wood 20 treated and the residual liquor contains the soluble reaction products so produced. The residual liquors, moreover, may be substantially free from products of degradation of cellulose, such as usually are present in relatively large amounts in the black liquor from the soda process. The constituents of the residual liquor, however, will differ somewhat according to the character of wood treated.
- 25 We have found that these residual liquors can advantageously be treated for the regeneration of further amounts of cooking liquor therefrom, for further use in the carrying out of the cooking operation. A part of the 30 residual liquor may be used directly without treatment, for admixture with regenerated liquor; or the residual liquor as a whole may in some cases be used over again, with additions of sodium sulfite or sodium thiosulfate 35 or both thereto before each successive cook if necessary.

Instead of using the residual liquor over again without treatment, we have found that this liquor can be treated in such a way that 40 a fresh amount of cooking liquor containing sodium sulfite and sodium thiosulfate can readily be produced therefrom. When the residual liquor from the pulp making operation is evaporated to dryness, and carbonized to destroy organic matter, and the resulting sodium compounds are dissolved in water, the resulting solution may contain some sodium thiosulfate, some sodium sulfite, and some sodium sulfide, some sodium sulfides 45 such as are known as polysulfides, some sodium carbonate and it may even also contain some sodium sulfate, particularly if subjected to oxidation during or after the carbonization. The nature and amounts of the different chemical compounds present will vary

somewhat with the conditions under which the carbonization is carried out, but particularly at high temperatures, complex reaction seems to take place between the complex organic substances in the product undergoing carbonization with the result that various sodium compounds containing sulfur are found in the solution obtained therefrom, among them frequently or commonly being sodium sulfide or sulfides and sodium thiosulfate. While the carbonization can be carried out at relatively low temperatures with avoidance or minimizing of sulfides and thiosulfates in the resulting solution, and while the solution produced by dissolving the sodium compounds from the carbonized product can be treated so as to obtain a reduction in the amount of thiosulfate present therein after sulfiting, we have found that such treatment is unnecessary and that some sodium thiosulfate may advantageously be present in the regenerated cooking liquor, when it contains sufficient sodium sulfite, and may advantageously be increased by converting sodium sulfide or polysulfides into additional thiosulfate by treatment with sulfur dioxide or sodium bisulfite or both, when the amount of thiosulfate is too small.

When the carbonized product from the carbonizing operation is in addition subjected to a smelting operation and the resulting smelted or molten material is dissolved in water or in aqueous solution to produce a solution of sodium compounds, varying amounts of sodium sulfides or polysulfides, and sodium thiosulfate, sodium sulfite, sodium sulfate, sodium carbonate, etc., may be present in the solution. If the amount of sodium sulfide or polysulfide is not too large, the solution may be treated directly with sulfur dioxide or sodium bisulfite or both for the conversion of such sulfides into sulfite, thiosulfate or both. Where a large amount of sodium sulfide or polysulfide is present in the solution of the dissolved sodium compounds, sodium sulfide may advantageously be converted into sodium sulfite, for example, by treating the solution first with carbon dioxide to drive off hydrogen sulfide and convert sodium sulfide into sodium carbonate or bicarbonate, and then by treating the carbonated solution or resulting solids or both with sulfur dioxide or sodium bisulfite or both to convert sodium carbonate or bicarbonate or both into sodium sulfite and to convert the remaining sodium sulfide if any into sodium sulfite or thiosulfate or both.

Accordingly the solution of the recovered sodium compounds recovered either from the carbonized product from the carbonizing operation, or from the melt from the smelter, after clarification if desired or necessary, can be treated with sulfur dioxide or with sodium bisulfite or both, and where these solutions contain proper amounts of sodium sulfide or

of polysulfide the treatment will result in the presence therein of additional sodium thiosulfate, in addition to whatever sodium thiosulfate may be present in the solution before such treatment. This treatment with sulfur dioxide or sodium bisulfite will also serve to convert sodium carbonate into sodium sulfite although some of the sulfite may be converted into thiosulfate. This treatment should ordinarily be continued until all of the carbonate has been sulfited. Some of the thiosulfate contents may be formed by the conversion of sodium carbonate into sodium sulfite and by reaction of the latter with elementary sulfur or with some of the loosely combined sulfur in the polysulfide when either or both of these is present, with the resulting production of sodium thiosulfate or some other compound which contains more sulfur than does the sodium monosulfite.

The method of carrying out the treatment of the residual liquors for the production of a further amount of cooking liquor therefrom, will be illustrated by the following more detailed description. It is one advantage of the invention that the process can advantageously be carried out in the equipment such as is now found in pulp mills constructed and operated for carrying out the soda process or the sulfate process with the addition of the necessary auxiliary equipment.

In general, the residual liquor may be evaporated in multiple effect evaporators until the concentrated liquor tests about 35 to 40° Bé. at 160 to 190° F.; then the hot concentrated liquor may be fed in regulated amounts into the back end of a rotary furnace such as is customarily employed in the soda process pulp mills, this rotary furnace being about 16 to 20 feet long and about 8 to 9 feet in diameter, and being lined with a good grade red brick. The rotary furnace may be provided with a suitable burner at the front end, for example an oil burner, so arranged that a long flame is projected into the rotary furnace, and so that the intensity of the flame can be controlled by adjusting the feed of fuel and air. The rotary furnace may be rotated at about 2 revolutions per minute. As the water is evaporated, the material is carried forward in the rotary furnace and the temperature becomes high enough to carbonize the organic matter and some volatile and combustible matter is given off from the material and may be ignited, thus helping to carry on the rotary furnace operation. Reducing the speed, for example, to one revolution per minute changes the operation to some extent, since volatile gases have a different opportunity to become ignited, as the material does not roll over so frequently as at the higher speed. By controlling the liquor feed and the flame at opposite ends of the rotary furnace, the ash can be delivered either in molten condition or as a well-burned ash, or as an underdone or

green ash. The ash may be melted quite easily in the furnace, and when molten gives off combustible gas. When the rotary furnace is running at good rate, producing a well-burned but granular ash, with little or no melting of ash in the rotary furnace, we have observed that a greenish yellow flame arose from the material within the furnace, especially along the upper surface and between the middle of the rotary furnace and the discharge or front end of the furnace. When the large amount of material in the lower part of the furnace rolled over, it sometimes extinguished this peculiar flame. This flame is apparently due to the liberation of elementary sulfur from the complex organic matter or sulfo-organic matter or perhaps from some thio-compound existing in the material undergoing decomposition, and to the burning of the elementary sulfur to sulfur dioxide. Sometimes the ash will continue to burn or to give off volatile and combustible gas even after it is discharged from the rotary furnace, this burning or combustion sometimes continuing for an appreciable period of time.

It is difficult to determine the exact nature of the chemical reactions which take place during such a carbonizing operation in such a rotary furnace; but analysis of the products produced indicates that a considerable amount of the combined sulfur existing in the residual liquor prior to decomposition by heat treatment may be driven off during the carbonization in the rotary furnace, the amount of sulfur thus being eliminated depending upon the manner in which the operations are conducted.

If the carbonized product from the rotary furnace is fed into a smelter, additional elimination of sulfur may take place. If the ash is allowed to oxidize, there may be a considerable amount of sodium sulfate in it; although by suitably reducing the material the amount of sulfate can be kept low. If a sulfate of sodium is added to the residual liquor before evaporation, or to the evaporated or dried products before carbonization, or to the smelter charge before smelting, an increased amount of sodium sulfide may be present in the smelted product, especially if a smelter is used.

We have examined some of the molten material from the rotary furnace, when the carbonizing operation was carried out so as to melt the charge, and our examination, after cooling, seems to show the presence of appreciable amounts of elementary sulfur, i. e., free and uncombined sulfur. Apparently the complex sulfo-organic compounds of the residual liquor decompose, in part at least, into sodium carbonate and liberate some sulfur in an uncombined state, this reaction perhaps being analogous to the decomposition of sodium thiosulfate under heat treatment.

The reactions which take place are, however, apparently quite complex and we do not wish to limit ourselves by any theoretical explanation of what the reactions may be.

5 In the treatment of the residual liquors for the regeneration of further amounts of cooking liquors therefrom, we find it desirable to prevent the building up of the sodium thiosulfate to an objectionable or excessive 10 degree. The amount of sodium thiosulfate can be regulated in part by suitable regulation of the carbonizing operation in the rotary furnace, and in part by proper treatment of the leach liquor obtained from the 15 ash discharged from such furnace. Some of the leach liquors obtained from the ash from such rotary furnace we have found to contain considerable percentages of sodium thiosulfate, even before the leached liquor was 20 sulfited. By controlling the rotary furnace operation, however, this amount can be regulated to a greater or lesser degree, apparently by elimination of sulfur therefrom which may be burned to sulfur dioxide. Some of 25 the sulfur may be eliminated during the smelting operation in a smelter if the ash from the rotary furnace is to be subjected to smelting. The sodium which would otherwise be present as sodium thiosulfate may be 30 present in the leached liquor in part as sodium sulfite or sodium sulfide or even as sodium carbonate.

The stack gases coming from the rotary furnace during the carbonizing operation 35 contain quite an amount of sulfur dioxide; and some of the sulfur dioxide may become further oxidized to sulfur trioxide. We have collected considerable amounts of solids from the flue between the rotary furnace and the 40 stack and found that under certain conditions these solids consisted largely of sodium sulfate. By scrubbing the stack gases with a solution containing sodium carbonate, a considerable portion of the sulfur compounds 45 escaping in the stack gases may be collected either as sodium sulfite, sodium thiosulfate, or sodium sulfate.

The ash discharged from the rotary furnace may be directly subjected to a leaching 50 operation, for example, by conveying it to a dissolving tank or leaching tank where the sodium compounds are leached away from the insoluble carbon. We have found that a good granular ash leached somewhat better 55 than an ash which contains a large percentage of molten material produced during the treatment in the rotary furnace. It is easier to clarify the leach liquor from the 60 granular ash and get a good cooking liquor therefrom quite free from suspended carbon. Accordingly, in carrying out the carbonization operation in the rotary furnace, the operation is advantageously regulated and controlled to avoid any large percentage of mol- 65 ten material and to produce a suitable prod-

uct of a granular character from which the sodium compounds can readily be leached, leaving the carbon behind.

The residual liquors from a pulp making operation in which the cooking liquor contains essentially normal sodium sulfite, without any appreciable amount of sodium thiosulfate, can similarly be treated according to the process of the present invention for the production of a cooking liquor containing both sodium sulfite and sodium thiosulfate. When such a residual liquor is evaporated to dryness and the dried residue carbonized in a rotary furnace, more or less of the sulfur-containing compounds of the product will be 70 decomposed and some sulfur separated therefrom. Varying amounts of the sodium contents of the carbonized product may be present as sodium carbonate, some of the sulfur originally combined with the sodium apparently having been driven off or converted into some other compound. Some of the sulfur-containing compounds, varying with the conditions under which the carbonization is carried out, will usually be converted into sodium sulfide or polysulfide, and appreciable amounts of sodium sulfide and polysulfide may be present in the carbonized product, particularly where the carbonization is carried out at higher temperatures and with 75 melting or fusion of the product.

In the carrying out of such a process, we have obtained a composite leach liquor in which sodium compounds were present in approximately the following ratio, namely, about 5 parts of sodium carbonate, about 4 parts of sodium sulfite, and about 1 part of sodium sulfide. In another case where the rotary furnace operation was carried out with a long flame and using hot strong liquor 80 directly from the evaporators, a well-burned granular ash was obtained, which showed approximately the following ratio, namely, about 75 parts of sodium carbonate, about 20 parts of sodium sulfite, and about 5 parts 85 of sodium sulfide.

Solutions of such compounds in the ratio above stated, after leaching away from carbon, and clarification in whole or in part when necessary, can be treated with sulfur dioxide gas, for example, by running the solution over an absorption tower, through which or into which sulfur dioxide is introduced. When such a liquor is sulfited in this way, it will contain a large amount of sodium sulfite, and will contain appreciable amounts of sodium thiosulfate, depending upon the amount of sodium sulfide and polysulfides present in the solution sulfited, and depending also upon the amount of sodium thiosulfate, if any, present in the solution before it is sulfited.

In examining the product, we have examined the melted material which was dug out of the rotary furnace after cooling and 130

found that it varied from black through grey and some of it was even pinkish in color in the interior of some of the lumps. In places there were appreciable amounts of yellow ma-

5 terial, appearing to be elementary sulfur. While the material was being treated in the rotary furnace, there was a thin flame which resembled burning sulfur. This flame occurred, however, only in the hot portion of  
10 the furnace and it is our opinion that some of the sulfur, originally present as sulfur-compounds in the residual liquor, is set free as elementary sulfur, or is converted into some other compound and volatilized during  
15 the rotary furnace operation. The fact that some sulfur is eliminated and some sodium carbonate is formed, indicates that carbon dioxide in some way replaces or displaces sulfur or a sulfur-containing radical to which  
20 the sodium is united. It may even be that some carbon directly displaces some sulfur, and may to some extent react with sulfur to form carbon bisulfide, although we do not limit ourselves by any such explanation of  
25 the actual reactions which go on.

In general it is advantageous to carry out the rotary furnace operation under regulated conditions which will retain as much as possible of the sulfur so that it can be recovered as sodium sulfite in the regenerated cooking liquor, without forming too much sodium sulfide and sodium sulfate. We have found it desirable to carbonize the dried material under regulated temperature and air  
30 conditions so as to avoid the production of excessive amounts of sodium sulfide and sodium sulfate, and also to avoid the presence of an excessive amount of sodium thiosulfate in the regenerated cooking liquor. By using  
35 a long oil flame fed in at the same end as the hot strong liquor, and carrying the flame and material in the same direction, excessive temperatures can be more readily avoided, and by regulating the temperature of such an  
40 operation and the amount of air, a large amount of sulfite can be directly recovered and made available in the regenerated cooking liquor.

Where the ash from the rotary furnace is  
50 not directly leached, but is subjected to smelting, the resulting melt from the smelter contains such a small amount of carbon that the solution of the sodium compounds of the melt may be separated from undissolved  
55 residue by decantation, and may be thereafter clarified when considered desirable.

As a step in the treatment of the solution produced by dissolving the melt or by leaching the ash from the carbonizing operation,  
60 we have found it advantageous to thoroughly mix a small amount of caustic soda with the liquor or solution, and then thoroughly mix in a small amount of magnesium sulfite. The resulting decomposition which occurs  
65 aids in the coagulation of suspended carbon

and facilitates the separation of a clarified liquor from the insoluble carbon and other insoluble materials.

In order to regenerate a cooking liquor from the leached liquor or from the solution of the molten material, such liquor or solution may be subjected, either directly or after further treatment, to a sulfiting operation or treatment. This treatment may be with sulfur dioxide or with an acid solution of sodium sulfite containing varying amounts of excess sulfur dioxide over and above that corresponding to the normal sodium sulfite. The sulfur dioxide, either introduced as such, or in an acid sulfite solution, will react with sodium carbonate, or bicarbonate, setting free carbon dioxide, and forming sodium sulfite. Sodium thiosulfate already present in the liquor or solution apparently remains substantially unchanged by this sulfiting operation. Sodium sulfide or polysulfides may react with sulfur dioxide or acid sulfite to produce additional amounts of sodium thiosulfate; and some thiosulfate may be formed by the reaction of sodium sulfite with sulfur present in the liquor as such or as polysulfide sulfur in the solution. Ordinarily, the proportion of sodium carbonate in the solution or leach liquor will be such that a prepondering amount of sodium sulfite will be directly produced, and the amount of sodium thiosulfate will be relatively low, especially when the carbonizing operation is properly conducted.

Where, however, the liquor prior to the sulfiting operation contains a large amount of sodium sulfides it may advantageously be subjected to a preliminary treatment before sulfiting in order to reduce the amount of sulfides which it contains. For this purpose it may be treated with carbon dioxide in sufficient amount to convert some of the sodium sulfide into a carbonate of sodium and liberate hydrogen sulfide gas. This gas may be burned to produce sulfur dioxide and the latter used in the production of the regenerated cooking liquor. By carbonation of the solution of the recovered sodium compounds in this way, prior to sulfiting, some of the sulfur is eliminated as hydrogen sulfide, thus reducing the amount of sodium sulfide in the liquor and correspondingly reducing the amount of thiosulfate which will be present in the liquor after the sulfiting treatment. By regulating the amount of carbonating to which the solution is subjected, the amount of thiosulfate subsequently present in the regenerated cooking liquor can be regulated; and part or all of the sodium which would otherwise be converted into sodium thiosulfate may be converted into a carbonate of sodium which upon subsequent sulfiting may be converted into sodium sulfite.

Analysis of the solution of the recovered

sodium compounds, or an actual sulfiting of a sample of the solution, followed by analysis, will show whether it is desirable to carbonate the solution prior to the sulfiting operation for the production of a regenerated cooking liquor.

The carbonating treatment, where this is desirable, may be carried out in different ways. One advantageous method which we have used successfully consists in introducing into the bottom of a tall tank containing the solution of the recovered sodium compounds, a strong solution of acid sodium sulfite, and causing this to react so that carbon dioxide displaces hydrogen sulfide from some of the sodium sulfide contained in the solution. That is, the acid sulfite will first tend to react with sodium carbonate to form bicarbonate and then react to set free carbon dioxide which will then displace hydrogen sulfide from some of the sodium sulfide of the solution. The thiosulfate already present in the solution may be increased in amount when desired, by additional thiosulfate produced from uncarbonated sulfides or produced from polysulfide sulfur or in any other suitable manner.

By regulating the carbonating operation, the amount of additional thiosulfate subsequently formed by the sulfiting operation can be regulated. If the carbonating treatment is omitted entirely, the maximum increased amount of thiosulfate may be formed; while if all or as much as possible of the sulfide is carbonated and converted into a carbonate of sodium, a lesser amount of additional thiosulfate may be formed; and any intermediate amount may be formed by regulating the carbonating operation prior to sulfiting.

In analyzing or testing the regenerated cooking liquor, we have found that good results can be obtained by titration with standard sulfuric acid solution using methyl-orange as an indicator for the purpose of determining the amount of active sodium sulfite, due allowance being made for any small amounts of other reactive sodium compounds, if any, which may be present. The other reactive sulfur compounds may be determined by the use of standard iodine solution, making allowance for the sodium sulfite determined as above. If the standard iodine solution were alone relied upon and the entire result computed as sodium sulfite ( $Na_2SO_3$ ), without allowing for the thiosulfate contents, there would be danger of the operator employing too little actual sodium sulfite and in some cases too much sodium thiosulfate in the cooking operation and this would result in the production of an unsatisfactory pulp, but by properly analyzing or testing the leach liquor or the solution of the melt when using a smelter, its composition can be determined and its treatment then regulated and controlled to give a regenerated cooking liquor

of suitable composition, containing a preponderating amount of the sodium sulfite and a smaller amount of the thiosulfate.

After extended investigation we have found it important in using such a regenerated cooking liquor for cooking additional charges of wood chips to employ enough actual sodium sulfite ( $Na_2SO_3$ ) to avoid the objectionable features of an excess of sodium thiosulfate ( $Na_2S_2O_3$ ) when used with too small an amount of sodium sulfite; since, if not enough sodium sulfite is employed, it is difficult or impossible to obtain a good quality and good color of pulp which can be satisfactorily and economically bleached by commercial bleaching methods.

Insofar as we are aware, it is broadly new to cook wood with such a cooking liquor containing a sufficiently large amount of sodium sulfite, the cooking liquor also containing some sodium thiosulfate. Satisfactory cooking of the wood chips can be effected with the sodium thiosulfate as an ingredient of the cooking liquor, and without the objection resulting from the use of an insufficient amount of sodium sulfite, accompanied by a large amount of sodium thiosulfate in the cooking liquor. We believe that we are the first to discover how to cook woods successfully with a solution containing essentially both sodium sulfite and sodium thiosulfate, either with or without a small amount of caustic soda, etc., so as to get pulp of a good quality which is economically bleachable by commercial bleaching methods. We also believe we are the first to treat a residual liquor from such a cooking operation for the production therefrom of further amounts of cooking liquor containing sodium sulfite accompanied by sodium thiosulfate. We believe we are also the first to show how the residual liquor can be treated so as to recover the sodium content and to regenerate a cooking liquor therefrom which contains a regulated amount of sodium thiosulfate together with a sufficient and preponderating amount of sodium sulfite.

In order to make up for losses of chemicals in the process, or to rectify or to further regulate and control the composition of the cooking liquor, additional amounts of suitable reagents may be added thereto. For example, additional sodium carbonate can be added to the solution which is to be sulfited, and sodium sulfite produced therefrom. So also, by using sodium bisulfite, or an acid sodium sulfite solution, for the sulfiting operation, the additional sodium sulfite thus added will increase the amount which the regenerated cooking liquor will contain. When the ash from the carbonizing operation is subjected to a smelting operation, additional sodium sulfate or bisulfate or both can be added at some time prior to the smelting operation, and some sodium sulfide can be produced therefrom. This sodium sulfide may be sul-

fited to the desired extent or the solution can first be subjected to carbonation to convert some of the sodium sulfide into a carbonate of sodium and drive off hydrogen sulfide, and 5 the sodium compounds may then be subjected to the sulfiting operation.

By properly regulating the treatment of the constituents of the residual liquor during carbonization, or during carbonization and 10 smelting, and by proper treatment of the resulting solution obtained from the carbonized product or from the melt obtained therefrom, regenerated cooking liquor can be produced of suitable composition for the further 15 carrying out of the pulp making operation.

This pulp making operation, as previously explained, is carried out with a cooking liquor (which may be regenerated from the residual liquor) containing a large amount of sodium sulfite, for example, amounting to 30% or more by weight of the bone dry weight of the wood, together with sodium thiosulfate. Insofar as we are aware, it is broadly new 20 in the pulp making art to subject wood to a cooking operation with a liquor containing both sodium sulfite and a regulated but smaller amount of sodium thiosulfate without caustic soda; and accordingly we claim the use of such a cooking liquor broadly as 25 well as the cooking of wood for the production of chemical pulp with such a composite cooking liquor. The cooking liquor need not, as hereinbefore explained, contain only sodium thiosulfate and sodium sulfite as it may 30 contain small and regulated amounts of sodium carbonate.

Where certain pines, such as those which contain a large amount of resinous constituents (especially the yellow pines of the 40 southern portion of the United States of America which are the main source of naval stores), are to be cooked with a cooking liquor which contains a large amount of sodium sulfite in conjunction with sodium thiosulfate, etc. for the production of chemical pulp, they may advantageously be given a regulated preliminary treatment for the purpose of removing a portion or all of the non-fibrous constituents which are readily soluble in a 45 suitable volatile solvent. Where desirable, the solution of the non-fibrous constituents in the volatile solvent may be subsequently treated so as to separate and reclaim the volatile solvent and permit the recovery of 50 the non-fibrous constituents.

This preliminary treatment of the wood, advantageously in the form of chips, should be carried out in such manner and under such 55 regulation that the undissolved non-fibrous constituents are left in a chemical and physical condition which will permit the resulting chips to be successfully treated with a cooking liquor such as referred to above, with the production of a suitable grade of chemical pulp. In particular, it is important to

avoid heating the chips to a temperature so high that the non-fibrous constituents are so changed chemically that they may not be readily made soluble in aqueous solution by cooking at elevated temperature and pressure 70 with a cooking liquor such as referred to above.

In general the treatment, prior to thorough impregnation of the wood chips with cooking liquor, should not be allowed to exceed about 75 100° C. The treating of wood chips with water alone at temperatures much above 100° C. so changes the chips that they can not readily be pulped with a solution containing essentially sodium sulfite and sodium thiosulfate without further treatment, for example, with caustic soda solution, and a similar action apparently takes place where the chips are heated above 100° C. before thorough impregnation. In certain cases, as where the digester charge of pine chips is heated rapidly to the cooking temperature, it may be desirable to cook the pine wood chips with a cooking liquor such as is referred to above, and thereafter to treat the resulting wood chips or the pulp obtained therefrom, with a liquor which contains a small amount of caustic soda or other suitable reagent such, for instance, as sodium sulfid which is capable of readily removing certain non-fibrous constituents which are not readily removable by cooking with a cooking liquor which contains 80 essentially sodium sulfite and sodium thiosulfate. The caustic soda etc. can be added, for example, near the end of the cook, or after 85 a partial cook, or a cooking liquor containing the caustic soda etc. can be used after the first liquor is drawn off.

We give below a few analyses of different 90 leach liquors obtained by dissolving the soluble sodium compounds contained in carbonized material or in molten material or mixtures thereof, and also analysis of a regenerated cooking liquor.

| Leached liquor                                |       | Grams per litre |
|-----------------------------------------------|-------|-----------------|
| NaOH                                          | ----- | .3              |
| Na <sub>2</sub> S                             | ----- | 3.8             |
| Na <sub>2</sub> SO <sub>3</sub>               | ----- | 15.75           |
| Na <sub>2</sub> S <sub>2</sub> O <sub>3</sub> | ----- | 99.935          |
| Na <sub>2</sub> CO <sub>3</sub>               | ----- | 120.97          |

| Leached liquor                                |       | Grams per litre |
|-----------------------------------------------|-------|-----------------|
| Na <sub>2</sub> CO <sub>3</sub>               | ----- | 53.66           |
| NaOH                                          | ----- | None            |
| Na <sub>2</sub> S                             | ----- | 8.77            |
| Na <sub>2</sub> S <sub>2</sub> O <sub>3</sub> | ----- | 2.37            |
| Na <sub>2</sub> SO <sub>3</sub>               | ----- | 2.42            |

| Regenerated liquor                            |       | Grams per litre |
|-----------------------------------------------|-------|-----------------|
| Na <sub>2</sub> SO <sub>3</sub>               | ----- | 169.9           |
| Na <sub>2</sub> S <sub>2</sub> O <sub>3</sub> | ----- | 21.33           |
| Na <sub>2</sub> CO <sub>3</sub>               | ----- | 5.74            |

The following is a suitable method of analysis for analyzing liquors of the character above indicated.

5 Total alkalinity. A 10 cc. sample of liquor is titrated with normal sulfuric acid using methyl orange as an indicator. This total alkalinity represents caustic soda, sodium carbonate, sodium sulfide and one-half the sodium sulfite.

10 Another 10 cc. sample is treated with excess barium chloride in a 250 cc. flask, made up to the mark with distilled water, the clear solution settled or filtered off and two aliquot portions of 50 cc. are taken. The alkalinity 15 on one 50 cc. aliquot portion is determined by titration with tenth normal sulfuric acid using methyl orange as an indicator. This alkalinity represents caustic soda and sodium sulfide. The resulting solution is then boiled 20 to drive off hydrogen sulfide and cooled and is then titrated with tenth normal iodine solution using starch as an indicator. This gives the sodium thiosulfate. The second 50 cc. aliquot part is titrated with tenth normal 25 ammoniacal zinc chloride solution using lead acetate paper as outside indicator. This gives the sodium sulfide.

The precipitate formed as above described by treating the 10 cc. sample with excess 30 barium chloride is filtered off and the precipitate washed with hot water. This precipitate of barium carbonate and barium sulfite is transferred to a beaker, distilled water added, then tenth normal iodine solution 35 added in excess of the possible sulfite content, the precipitate then dissolved in diluted hydrochloric acid, starch solution added, and the solution titrated with tenth normal sodium thiosulfate. The difference between the 40 tenth normal thiosulfate reading and the tenth normal iodine reading represents the sodium sulfite ( $Na_2SO_3$ ).

The amount of sodium carbonate is determined by subtracting the amount of caustic 45 soda, sodium sulfide, and half the sodium sulfite from the total alkalinity.

The following description of operations on various woods with a cooking liquor such as referred to herein will serve to show how the 50 process may be operated in practice with good results. An unlined welded digester, of the stationary, vertical type, the capacity of which was about 1,900 cubic feet, was filled with jack pine chips. These chips were obtained by barking sticks of two foot length 55 jack pine (*Pinus divaricata* or *Banksiana*), then chipping and screening so as to get fairly uniform chips of about  $\frac{3}{8}$  to  $\frac{5}{8}$  inch in length along the grain. The chips contained 60 about 10 to 20% moisture. About 7,500 gallons of regenerated cooking liquor was used in a digester charge. About 9,000 pounds of sodium sulphite was contained in about 6,000 gallons of fresh regenerated cooking liquor, 65 which we call white liquor, and there was

also added about 1,500 gallons of residual liquor from the process which we call red liquor, the amount of unused sodium sulphite and sodium thiosulphate in the red liquor being undetermined. The white liquor contained about 1,000 pounds of sodium thiosulphate in some instances, while in other instances the amount was sometimes less and sometimes more than this.

70 The digester was sealed up and then steam introduced into the digester slowly and gradually, at the same time causing the cooking liquor to circulate throughout the body of chips so as to give them substantially uniform treatment. About three to five hours was taken in heating the digester charge from about 20 deg. cent. up to about 180 to 190 deg. centigrade. The contents of the digester were maintained at this high range of temperature for about seven to fifteen hours. Sometimes the digesters were held for a longer time than fifteen hours and sometimes for a shorter time than seven hours.

75 We have found that by providing a false bottom in the digesters, and suitable piping and pumps so that the cooking liquor can be withdrawn from beneath the false bottom and circulated in copious amount and discharged into the upper portion of the digester above the wood chips so that the cooking liquor is quite uniformly spread out above the entire body of chips and caused to percolate in a substantially uniform manner downward through the body of chips, and the liquor is progressively heated during its 80 passage from the bottom to the top of the digester, splendid results may be readily obtained.

85 As an aid in determining when the cooking operation has progressed to the desired degree, a sampling device may be installed at one or more places in the side of the digester, through which samples of stock may be drawn from time to time. So also thermometers may be installed at various points.

90 Other digesters of the same size and kind, provided with the same type of circulation equipment, were filled in some instances with wood chips obtained from barked aspen (northern poplar) and in other instances from barked white birch. The same volume 95 of cooking liquor and substantially the same composition as was used on the jack pine chips, was used satisfactorily in cooking the non-coniferous woods. In these various instances, splendid chemical pulp of very light color in the unbleached condition, was obtained. We found, however, that the time 100 taken for heating the digester contents when aspen or birch were being cooked, as well as the time during which the contents were held at the higher range of temperature, could be materially reduced from that which was found necessary or desirable with the jack pine.

70

75

80

85

90

95

100

105

110

115

120

125

130

While the cooking liquor charges referred to above contained about 9,000 pounds of sodium sulfite, we have found by actual operations that the amount of chemicals can be 5 very much reduced from that figure. The better and more uniform the circulation, the lower the amount of chemicals may be, within reasonable limits. The higher the concentration of the chemicals, and especially 10 of sodium sulfite, in the cooking liquor, the more active the cooking operation, also within reasonable limits. The higher the temperature, the more active the cooking liquor becomes, but we have found that it is not 15 advisable to cook coniferous woods at a temperature much below 180° C. and we prefer that the temperature be even higher than this, for example up to 190° C. At temperatures much higher than this, the digester and 20 boiler strength required entails considerable additional expense, while if the cooking temperature be too low, the time required is needlessly long.

Non-coniferous woods, in general, are more 25 easily pulped by this process than are the coniferous woods, as a general class.

The chemical pulps obtained from woods by this process are capable of being made into very strong papers, possessing light 30 color, even when unbleached.

The pulps obtained by this process from various woods, for example aspen and birch, may be made into unbleached papers which are lighter in color than papers made with 35 chemical pulp from the same woods when cooked by either the soda process or the sulphate process, when the same kind of treatment in the paper making operation is given to them. And with the same kind of treatment, the papers are stronger than those obtained by the other processes referred to, if the same lightness in color is obtained in the unbleached and uncolored papers. That is to say, that with this new process new kinds of 40 45 papers may be produced from the unbleached and uncolored pulps which are characterized by relatively greater strength. For instance, paper made from a fibre furnish of 100% aspen pulp, obtained by this process, being 50 unbleached but having a small amount of blue color added to the stock in the beater, was made in weights ranging from 30 pounds to 60 pounds, for example, per ream of 480 sheets each 24" x 36", which showed a bursting 55 strength when tested by the Mullen tester of from three-fourths to over a point a pound. Similar papers were made from 100% white birch pulp from this process which tested relatively higher than the similar paper made 60 from the aspen pulp. Similar papers made from 100% fibre furnish of jack pine pulp obtained by this process showed bursting strength of from one to as high as one and a half points per pound. Some have tested 65 considerably higher than this, depending up-

on the cooking conditions and also upon the subsequent treatment which the stock received.

These pulps being very light in color, especially when washed with hot water after removal of the residual liquor, may readily be used for light colored papers or may even be tinted or colored to almost any desired shape, even without the pulp having been bleached. The papers referred to above were made on a Fourdrinier machine, with 70 mesh wire, operating at 300 feet or more per minute. The wire was 118 inches wide.

We have stated above that the chemical pulps obtained from woods by this pulp making process may as a general class be bleached by the usual bleaching methods. However, we have found that where a particular grade of bleached pulp is desired, the pulp, after washing, preferably with hot water, may be advantageously treated with chlorine in the presence of water and at ordinary temperature so as to convert a substantial portion of the non-fibrous material into bleached, oxidized or chlorinated compounds, depending upon the character of the various constituents. These treated pulps may then be washed or otherwise treated to remove water soluble compounds and the resulting pulp given a further treatment with a solution of bleaching powder. A small amount of caustic soda may be added to the bleaching powder solution, if desired, for the purpose of increasing the amount of available alkali therein.

The method of bleaching chemical pulps is more fully-described in one of our earlier patent applications. By using this method of bleaching chemical pulps which are characterized by high white and relatively great strength may be obtained and thus permit the production of paper of high white and improved strength. This refers not only to pulps obtained from coniferous woods but also and particularly to pulps obtained from non-coniferous woods.

We have found that this method of bleaching is useful for the bleaching of chemical pulps obtained from woods which in their natural state contain considerable quantities of tanning materials, dyestuffs or other coloring matters which might otherwise interfere with the production of high white and the retention of strength.

We have found that by subjecting these chemical pulps at high density, for example from 15% to 25%, to the action of a solution of bleaching powder at temperatures around 80 to 100 deg. F., during agitation or conveying or mixing by means of large size screw or worm conveyors, the pulps may be made "slower" prior to their treatment in a beating engine. The unbleached pulps may be treated in this way, without using bleaching solution to make them "slower" thus aiding

in the production of unbleached papers of superior quality.

It will thus be seen that the invention provides a new pulp making process in which 5 the wood is cooked with a cooking liquor containing a mixture of sodium sulfite and sodium thiosulfate to produce a satisfactory chemical pulp; as well as an improved and distinctive residual liquor which may be advantageously treated to regenerate further 10 amounts of cooking liquor therefrom for further use in the cooking operation.

The process of the present invention accordingly presents many advantages, among 15 which may be mentioned the following; it enables a good yield of new and improved pulps to be obtained even from the usual pulp woods; it enables a relatively high yield of satisfactory chemical pulp to be obtained 20 from various woods which are not ordinarily considered to be pulp woods; it can be carried out in existing mills utilizing some of the existing equipment, and requires but moderate change in such mill construction; 25 the cooking liquors can be regenerated from the residual liquors by novel and improved methods of treatment; and the pulps have new and distinctive properties and can be bleached for the production of high grade 30 pulp.

While sodium has been used as the alkali in this case, we do not wish to exclude the use of other alkali compounds where their use is economically justified.

35 We claim:

1. The method of producing pulp from wood which comprises subjecting the same to a cooking operation under pressure and at an elevated temperature with a cooking 40 liquor free from alkali hydroxide and containing substantial amounts of a sulfite of an alkali and a thiosulfate of an alkali, the cooking liquor being supplied with an adequate amount of alkaline reactive compound to 45 maintain the liquor alkaline to litmus until the end of the cooking operation, at least one-half of the alkali content of the cooking liquor being supplied as sulfur-bearing compounds and the amount of alkali supplied as 50 a sulfite being at least as large as the amount supplied as a thiosulfate.

2. The method of producing pulp from wood which comprises subjecting the same to a cooking operation under pressure and at 55 an elevated temperature with a cooking liquor free from alkali hydroxide and containing substantial amounts of sodium sulfite and sodium thiosulfate, the amount of sodium sulfite being in excess of about 29% 60 by weight of the bone dry weight of the wood cooked, and the amount of sodium sulfite being larger than the amount of sodium thiosulfate, and sufficient to maintain the liquor alkaline to litmus throughout the cooking 65 operation.

3. The method of producing pulp from wood which comprises subjecting the same to a cooking operation under pressure and at an elevated temperature with a cooking liquor free from alkali hydroxide and alkali sulfide 70 and containing substantial amounts of sodium sulfite and sodium thiosulfate and also containing a carbonate of sodium, the cooking liquor being alkaline to litmus, continuing the cooking operation until the fibres are readily separable from each other, the cooking liquor being supplied with an adequate amount of alkaline reactive sodium compounds to maintain the liquor alkaline to litmus until the end of the cooking operation, the amount of sodium sulfite being larger than the amount of sodium thiosulfate and at least one-half of the sodium content of the cooking liquor being supplied as sodium-sulfur compounds. 75

4. The method of producing pulp from wood which comprises subjecting the same to a cooking operation under pressure and at an elevated temperature with a cooking liquor containing substantial amounts of a sulfite of an alkali and a thiosulfate of an alkali, and subjecting the resulting product to a further cooking operation with a cooking liquor containing caustic alkali. 80

5. The method of producing pulp from wood which comprises subjecting the same to a cooking operation under pressure and at an elevated temperature with a cooking liquor containing substantial amounts of a sulfite of an alkali and a thiosulfate of an alkali, a caustic alkali being added during the latter part of the cooking operation. 95

6. The method of producing pulp from resinous woods which comprises gradually heating a digester charge of the wood to the cooking temperature with a cooking liquor substantially free from caustic soda and sodium sulfide and containing substantial amounts of a sulfite of an alkali and a thiosulfate of an alkali to effect impregnation of the wood with the cooking liquor before the cooking liquor reaches a temperature of 125° C., and thereafter raising the temperature and continuing the cooking operation, the cooking liquor being supplied with more alkali in the form of a sulfite of an alkali than in the form of a thiosulfate of an alkali. 105

7. The method of producing pulp from resinous wood which comprises subjecting the same to a thorough impregnation at a temperature below the active cooking temperature with a cooking liquor free from alkali hydroxide, alkali sulfide, and alkali carbonate and containing substantial amounts of a sulfite of an alkali and a thiosulfate of an alkali, and subsequently raising the temperature and subjecting the same to a cooking operation under pressure and at a temperature in excess of 155° C., at least one-half 110 of the alkali content of the cooking liquor 115

being supplied as alkali-sulfur compounds of which more is supplied as a sulfite of an alkali than as a thiosulfate of an alkali.

8. The method of producing pulp suitable for being converted into paper from resinous wood which comprises subjecting the wood to a preliminary impregnation with a cooking liquor, alkaline to litmus, containing substantial amounts of a sulfite of an alkali and a thiosulfate of an alkali and also containing a carbonate of an alkali but being free from alkali hydroxide, at a temperature below 155° C. and subsequently cooking the wood at a higher temperature and pressure, the liquor being supplied with sufficient alkaline reactive compounds to maintain the liquor alkaline to litmus until the wood fibers are rendered readily separable from each other, the cooking liquor being supplied with more alkali in the form of a sulfite of an alkali than in the form of a thiosulfate and at least one-half of the alkali content of the cooking liquor being supplied as alkali-sulfur compounds.

23 9. The method of producing pulp from heavy hardwood such as birches, maples, oaks, etc., which comprises charging the digester with the wood chips and with a cooking liquor free from alkali hydroxide and containing substantial amounts of sodium sulfite and sodium thiosulfate, the amount of sodium sulfite being in excess of about 30% by weight of the bone dry weight of the wood charged, and heating the digester charge to the cooking temperature, and cooking the charge until the fibers are rendered readily separable from each other, the cooking treatment being carried out by means of a liquor containing more sulfite than thiosulfate of sodium.

43 10. In the preparation of chemical pulp, the use of a cooking liquor free from alkali hydroxide and comprising sodium sulfite and sodium thiosulfate in substantial amount, the quantity of the sulfite being adequate to prevent the fibrous material being unduly impaired for paper making, due to the presence of the sodium thiosulfate, and at least one-half of the sodium content of the cooking liquor being supplied as sodium-sulfur compounds.

53 11. The method of producing pulp from wood which comprises subjecting the same to a two-stage cooking operation, the cooking liquor during the first stage containing a sulfite of an alkali and a thiosulfate of an alkali and the cooking liquor during the second stage containing a caustic alkali.

63 12. The method of producing pulp from coniferous woods which comprises charging the digester with the wood chips and with the cooking liquor free from alkali hydroxide and containing substantial amounts of sulfite of an alkali and a thiosulfate of an alkali, gradually heating the digester charge to the

cooking temperature over a period of about three to five hours, and carrying out the cooking operation thereafter at a temperature of about 180° to 190° C. and continuing the digestion with such cooking liquor supplied with sufficient alkaline reactive material to maintain the liquor alkaline to litmus until the fibers are rendered separable from each other, the amount of an alkali supplied to the cooking liquor as a sulfite being more than that supplied as a thiosulfate.

70 13. The method of producing pulp from wood which comprises subjecting the same to a cooking operation under pressure and at an elevated temperature with a cooking liquor free from alkali hydroxide and containing substantial amounts of a sulfite of an alkali and a thiosulfate of an alkali, said cooking liquor also containing residual liquor resulting from cooking another portion of the wood with such a liquor, the cooking liquor being supplied with sufficient alkaline reactive material to maintain the liquor alkaline to litmus until the fibers are rendered separable from each other, the amount of alkali supplied as a sulfite being more than that supplied as a thiosulfate.

80 14. The method of producing pulp from wood which comprises subjecting the same to a cooking operation under pressure and at an elevated temperature with a cooking liquor free from alkali hydroxide and containing substantial amounts of a sulfite of an alkali and a thiosulfate of an alkali, separating resulting residual liquor from fiber-bearing material, supplying sodium sulfite to such residual liquor and using the resulting liquor to cook fiber-bearing material containing organic matter including cellulose so as to solubilize organic matter thereof.

90 15. The method of producing pulp from wood which comprises subjecting the wood to a two-stage cooking treatment, first with a cooking liquor containing sodium sulfite and a sodium thiosulfate and then with a cooking liquor containing sodium sulfide.

100 16. The method of producing pulp from wood which comprises subjecting the wood to a two-stage cooking operation, the first stage including cooking the wood with a cooking liquor including sodium sulfite and sodium thiosulfate, the second stage including cooking the resulting product with a liquor including sodium sulfide and sodium carbonate, separating residual liquor from the fibrous material, subjecting the residual liquor to evaporation to dryness and to carbonizing or carbonizing and melting, dissolving the sodium salts from the resulting product, subjecting a part of the resulting solution to a sulfiting treatment and utilizing the sulfited liquor in the first stage of a similar pulp producing operation and utilizing the sodium sulfide, present in the unsulfited portion of

75

80

85

90

95

100

105

110

115

120

125

130

the solution, in the second stage of such latter operation.

17. The method of digesting woody material which includes subjecting such material to impregnation with a liquor free from alkali hydroxide and including substantial quantities of alkali sulfite, alkali thiosulfate and alkali carbonate, and subsequently raising the materials to a suitable higher temperature,

10 whereby the fibers are rendered sufficiently separable from each other to be desirable for paper making, said sulfite being present in sufficient quantity to overcome the tendency of the thiosulfate to impair the fibers for paper making which occurs when an insufficient quantity of sulfite is present in such a liquor, and the amount of alkali present as a sulfite being larger than that present as a thiosulfate.

15 18. The method of digesting woody material which comprises subjecting said material to heating in the presence of a liquor which includes residual liquor from a previous similar cooking operation and being free from alkali hydroxide and containing a thiosulfate and a sulfite of sodium in a sufficiently large quantity to substantially avoid otherwise undesirable effect of said thiosulfate, and subsequently subjecting the resulting 20 product to digestion at a higher temperature, whereby the fibers are rendered separable and desirable for paper making, the liquor being supplied with sufficient alkaline reactive material to maintain the liquor alkaline to litmus until the fibers are rendered separable, and the amount of sodium sulfite being larger than the amount of sodium thiosulfate.

25 19. In a process of treating lignified fibrous material to render the fibers more readily separable from each other and in which a substantial amount of loosely combined sulfur is present in a liquor utilized for treating such material and existing in a condition, such for instance as an alkali thiosulfate, capable of impairing the fibrous material for paper making, the steps which include supplying to the fibrous material in the presence of water and in the absence of an alkali hydroxide, sodium sulfite in an amount which is capable of counteracting the tendency toward impairment by such loosely combined sulfur, and whereby there is produced, as a result of the process, fibrous material comprising fibers separable from each other and suitable for conversion into paper, the amount of alkali supplied as a sulfite being more than that supplied as a thiosulfate and at least one-half of the alkali being supplied to the cooking liquor in the form of sodium sulfite.

30 20. As a new product, residual liquor resulting from digesting lignified fibrous material until the fibers are separable from each other and suitable for being converted into paper, by means of liquor including sodium

sulfite and sodium thiosulfate, such residual liquor being free from alkali hydroxide and including non-fibrous constituents derived from such material and including sodium sulfite in amount sufficient to counteract such tendency as the thiosulfate may have had for rendering the fibrous material undesirable for paper making, while the residual liquor was in contact with the fibrous material.

35 21. In a process of treating lignified fibrous material to render the fibers more readily separable from each other and in which a substantial amount of loosely combined sulfur is present in a liquor utilized for treating such material and existing in a condition, such for instance as an alkali thiosulfate, capable of impairing the fibrous material for paper making, the steps which include supplying to the fibrous material in the presence of water and in the absence of alkali hydroxide, sodium sulfite in an amount which is capable of counteracting the tendency toward impairment by such loosely combined sulfur and whereby there is produced, as a result of the process, fibrous material comprising fibers separable from each other and suitable for conversion into unbleached paper, and subsequently bleaching the fibers by subjecting them to the action of an active

40 reagent including chlorine, in the presence of water, separating resulting liquor from the resulting fibrous material, and subsequently subjecting such material to an oxidizing bleaching treatment, whereby the fibers are obtained in a bleached condition suitable for being converted into white paper.

45 22. The method of obtaining fibrous material suitable for paper making, which includes digesting lignified fibrous material by means of cooking liquor that is free from alkali hydroxide and is supplied with a substantial amount of a sulfite of sodium, a substantial but lesser amount of a thiosulfate of sodium and with a regulated amount of another reactive compound capable of digesting a substantial amount of the non-fibrous constituents in such material, and terminating the digestion when the fibers have been rendered separable from each other to the desired degree, the liquor being supplied with a sufficient amount of a sulfite of sodium to substantially prevent loosely combined sulfur of the thiosulfate blackening the fibers to such a degree that they are rendered and remain unsuitable for conversion into light colored papers.

50 23. The method of digesting wood, which includes subjecting wood chips to a digestion operation at elevated temperature by means of a liquor that is free from alkali hydroxide and is supplied with a substantial amount of a sulfite of an alkali, a substantial but lesser amount of a thiosulfate of an alkali, and with a sulfid of an alkali in an amount less than that of the sulfite of an alkali but adequate

70

75

80

85

90

95

100

105

110

115

120

125

130

to effect digestion of a substantial amount of the non-fibrous constituents of the woody material and whereby, as a result of this process, fibrous material is obtained which is 5 suitable for paper making.

24. The regenerative process of obtaining fibrous material suitable for paper making, which includes digesting lignified fibrous material by means of cooking liquor free from 10 alkali hydroxide and including a substantial amount of sodium sulfite and a substantial but lesser amount of sodium thiosulfate until a sufficient amount of the non-fibrous constituents of such material have been digested 15 so as to render the fibers separable from each other to the desired degree, thereby producing a residual liquor, at the termination of the digestion, which is alkaline to litmus and which contains sodium sulfite in amount sufficient to counteract the tendency of the thiosulfate to blacken the fibrous material, terminating the digestion without permitting the fibrous material to become impaired for paper making, separating residual liquor 20 from the fibrous material, removing water from the other ingredients of the residual liquor, furnacing sodium organic compounds in the concentrate to produce an alkali-containing product which includes more sulfur-free alkali compound as compared to sulfur-containing alkali compound than did the residual liquor from which it was derived, subsequently forming a cooking liquor including alkali-containing material derived 25 therefrom and employing such cooking liquor in the digestion of lignified fibrous material.

25. The two-step process of obtaining pulp, which includes subjecting lignified fibrous material to treatment at elevated temperature by means of liquor supplied with a substantial amount of a sulfite of an alkali and a thiosulfate of an alkali, and thereafter subjecting the resulting fibrous 25 material to treatment by means of liquor supplied with alkali hydroxide and alkali sulfide.

26. The method of producing pulp from resinous wood which comprises subjecting such wood by means of a volatile resin solvent to a preliminary extraction to extract resinous matter at a relatively low temperature and subsequently treating the remaining fiber-bearing material at a higher temperature and under elevated pressure with a liquor free from alkali hydroxide and containing an alkali thiosulfate and a sulfite of an alkali until a substantial portion of the non-fibrous organic constituents thereof have been solubilized.

27. The method of producing pulp from wood which comprises subjecting the wood to a cooking operation at an elevated temperature with a non-acid cooking liquor free from alkali hydroxide and alkali sulfide and consisting essentially of sodium monosulfite

and sodium thiosulfate, the amount of sodium monosulfite being larger than the amount of sodium thiosulfate and sufficient to maintain the liquor alkaline to litmus throughout the cooking operation.

28. The method of producing pulp from wood which comprises subjecting the wood to a cooking operation at an elevated temperature with a cooking liquor free from alkali hydroxide and consisting essentially of sodium sulfite in amount not less than 30% of the bone dry weight of the wood and of sodium thiosulfate in amount not greater than 15% of the bone dry weight of the wood, the amount of sodium sulfite being sufficient to maintain the liquor alkaline to litmus throughout the cooking operation.

29. The method of producing pulp from wood which comprises subjecting the wood to a two-stage cooking operation, the first stage comprising a treatment with a cooking liquor comprising monosulfite of sodium, and the second stage comprising a treatment with a liquor comprising sodium sulfide.

30. The method of treating fiber-bearing material containing cellulose and other organic matter, which comprises subjecting wood to a digesting treatment under pressure at an elevated temperature by means of a cooking liquor containing a substantial amount of a monosulfite of an alkali and a lesser but substantial amount of a thiosulfate of an alkali; subsequently supplying to fiber-bearing material, derived from the wood and containing organic matter including cellulose, an alkaline compound capable of solubilizing some of such organic matter, and treating the fiber-bearing material with the resulting alkaline liquor containing the alkaline compound so as to obtain at the termination of such treatment an alkaline liquor which includes dissolved matter derived in part from such organic matter.

31. In the treatment of cellulosic fiber-bearing material, the use of a cooking liquor comprising a monosulfite of an alkali metal and a thiosulfate of an alkali metal in substantial amounts, the cooking liquor being free from any substantial amount of alkali hydroxide and the quantity of alkali metal supplied as a sulfite being more than that supplied as a thiosulfate and the amount of sulfite being sufficient to overcome tendency toward blackening of the fibrous material due to the thiosulfate.

32. The method of treating wood which comprises the following steps: (a) subjecting wood to a digesting treatment under pressure and at an elevated temperature by means of cooking liquor containing a substantial amount of a monosulfite of an alkali metal so as to solubilize a substantial portion of organic matter thereof; (b) subsequently supplying to fiber-bearing mate-

rial, derived from the wood and containing organic matter including cellulose, an alkaline sodium compound capable of solubilizing some of such organic matter, and 5 treating the cellulose-containing material with the resulting alkaline liquor so as to obtain at the termination of such treatment an alkaline liquor which includes dissolved matter derived in part from such organic 10 matter; and (e) subsequently washing fibers derived from the wood.

33. As a new product, an easily bleachable wood pulp of light color having separable fibers in a substantially unimpaired condition suitable for being converted into paper and having been obtained by the cooking of wood with a cooking liquor free from alkali hydroxide and containing essentially sodium sulfite and sodium thiosulfate, which is maintained 15 alkaline to litmus by means of alkaline sodium compounds throughout the cooking operation, such fibers being substantially free from dark colored reaction products due to loosely combined sulfur and reactive organic matter.

34. As a new product, an easily bleachable wood pulp of light color having separable fibers in a substantially unimpaired condition suitable for being converted into paper and 20 having been obtained by the cooking of long fibered wood with a cooking liquor that is free from alkali hydroxide and contains carbonate of sodium, sodium sulfite and a lesser amount of sodium thiosulfate, which is maintained 25 alkaline to litmus by means of alkaline sodium compounds throughout the cooking operation, such fibers being substantially free from dark colored reaction products due to loosely combined sulfur and reactive organic matter.

35. As a new product, an easily bleachable wood pulp of light color having separable fibers in a substantially unimpaired condition suitable for being converted into paper and 45 having been obtained by the cooking of short fibered wood with a cooking liquor that is free from sodium hydroxide in any substantial amount and contains carbonate of sodium, sodium sulfite and sodium thiosulfate, which is maintained 50 alkaline to litmus throughout the cooking operation, such fibers being substantially free from dark colored reaction products such as are produced when an insufficient amount of sulfite is present with 55 the thiosulfate.

36. The method of producing pulp from wood, which comprises subjecting the wood to a cooking operation with a cooking liquor that is free from alkali hydroxide and contains 60 essentially a sulfite of an alkali, separating resulting residual liquor from resulting fiber-bearing material, treating such residual liquor to decompose organic matter thereof and to form a regenerated cooking liquor that is free from alkali hydroxide and

contains essentially a sulfite of an alkali, admixing such regenerated cooking liquor with residual liquor resulting from a cooking operation such as first mentioned in this claim so as to form a cooking liquor containing 70 more alkali in the form of a sulfite of an alkali than in the form of a thiosulfate of an alkali, and using such cooking liquor in a digesting treatment of wood.

37. The method of treating wood, which comprises the following steps: (a) subjecting the wood to a digesting treatment under pressure and at an elevated temperature by means of cooking liquor containing a substantial amount of sodium monosulfite so as to solubilize a substantial amount of such organic matter by means of such sulfite; (b) subsequently supplying sodium sulfide to fiber-bearing material, derived from the wood and containing organic matter including cellulose, and treating the fibre-bearing material with the resulting alkaline liquor including sodium sulfid so as to obtain at the termination of such treatment an alkaline liquor which includes dissolved organic matter derived from the fibre-bearing material.

38. The method of treating wood, which comprises the following steps: (a) subjecting the wood to a digesting treatment under pressure and at an elevated temperature by means of cooking liquor containing a substantial amount of sodium monosulfite so as to solubilize a substantial portion of the wood by means of such sulfite; (b) subsequently supplying alkaline material including sodium carbonate to fiber-bearing material, derived from the wood and containing organic matter including cellulose, and treating the fibre-bearing material with the resulting alkaline liquor including sodium carbonate and a reducing sulfur-bearing compound of sodium so as to solubilize a portion of such organic matter.

39. The method of treating wood, which comprises subjecting the wood to a digesting treatment by means of cooking liquor that is free from alkali hydroxide and contains essentially a monosulfite of an alkali metal so as to solubilize organic matter thereof, subsequently adding to fiber-bearing material derived from the wood an alkaline liquor comprising sodium sulfide, and treating such fiber-bearing material therewith until some organic matter thereof has been solubilized.

40. The method of making pulp from lignified fiber-bearing material, which comprises digesting the material with a solution containing a sulfite of an alkali metal and a thiosulfate of an alkali metal, the solution being free from alkali hydroxide and from alkali sulfide and being further characterized by having substantially more alkali metal present as a sulfite than as a thiosulfate and the quantity of sulfite of alkali metal being sufficient to provide the solution, throughout

the digesting step, with an amount of such sulfite that is adequate to prevent blackening of the fibres by means of loosely combined sulfur present in the thiosulfate.

5 41. The method of making pulp from lignified fiber-bearing material, which comprises digesting the material with a solution containing sodium monosulfite and sodium thiosulfate, the solution also containing  
10 carbonate of sodium but being free from alkali hydroxide, and the solution being further characterized by having substantially more sodium present as sodium monosulfite than as sodium thiosulfate and the quantity  
15 of sodium monosulfite being sufficient to provide the solution, throughout the digesting step, with an amount of such monosulfite that is adequate to surmount and overcome the tendency of the thiosulfate to darken the  
20 fibers.

42. The method of treating lignified fiber-bearing material which comprises the following steps: (a) subjecting the material to a digesting treatment under pressure and at  
25 an elevated temperature by means of cooking liquor that is free from alkali hydroxide and contains essentially sulfite of sodium, thereby producing a residual liquor that contains sodium-sulfur-organic compounds; (b) evaporating water from the residual liquor;  
30 (c) furnacing sodium-sulfur-organic compounds therefrom under reducing conditions to produce a furnace product that contains sodium carbonate and sodium sulfide; (d)  
35 treating this furnace product with water to dissolve the sodium carbonate and sodium sulfide, thereby forming an alkaline solution; and (e) treating fiber-bearing material resulting from step (a) by means of the solution mentioned in step (d) thereby dissolving some of the organic matter present in the fiber-bearing material.

40 In testimony whereof we affix our signatures.

45 LINN BRADLEY.  
EDWARD P. McKEEFE.